

Dec. 13, 1932.

J. L. HERMAN

1,890,463

METAL COATED IRON OR STEEL ARTICLE AND METHOD  
AND APPARATUS FOR PRODUCING SAME

Filed April 3, 1931

2 Sheets-Sheet 1



Inventor:  
Joseph L. Herman  
By: Chas. Malcomte, Jr.

Dec. 13, 1932.

J. L. HERMAN

1,890,463

**J. L. HERMAN**  
**METAL COATED IRON OR STEEL ARTICLE AND METHOD**  
**AND APPARATUS FOR PRODUCING SAME**  
Filed April 3, 1931 2 Sheets

Filed April 3, 1931 2 Sheets-Sheet 2



Inventor.  
Joseph L. Herman  
By Frank A. O'Boyle Attw.

## UNITED STATES PATENT OFFICE

JOSEPH L. HERMAN, OF PEORIA, ILLINOIS, ASSIGNOR TO KEYSTONE STEEL & WIRE COMPANY, OF PEORIA, ILLINOIS, A CORPORATION OF ILLINOIS

METAL COATED IRON OR STEEL ARTICLE AND METHOD AND APPARATUS FOR PRODUCING SAME

Application filed April 3, 1931. Serial No. 527,496.

This invention has reference to metal coated iron or steel articles and to the method and apparatus for producing the same.

The invention has for its principal object 5 the coating of an iron or steel article with zinc so that the resulting article, whether it be wire, strips or the like shall possess a zinc coating of uniform thickness throughout and if wire, circumferentially and longitudinally 10 thereof, which coating will withstand severe deforming without flaking or peeling.

The invention has for a further object to coat iron or steel articles with a uniform thickness of zinc coating throughout and to 15 heat-treat the zinc coated article whereby to provide an effective bond between the zinc and the iron or steel base thereby allowing for severe deforming of the coated articles without flaking or peeling; the method of 20 heat treating employed inhibiting in part, if not wholly, the formation of zinc oxide on the surface of the zinc coating during the heat-treatment and also inhibiting to a considerable degree the formation of zinc oxide 25 skimmings on the surface of the molten zinc at the point where the articles treated and coated leave the bath, both of which are undesirable.

Other and further objects will more fully 30 appear from the following description.

That the invention may be more fully understood, reference is had to the accompanying drawings forming part of this description, illustrating a preferred embodiment 35 of the invention, in which:—

Fig. 1 is a side elevation, on a greatly reduced scale, of a unit by which my invention may be practiced;

Fig. 2 is a vertical sectional view, on a much 40 larger scale, showing the details of construction, of the unit, and

Fig. 3 is a cross-section, in plan, as the same would appear if taken on the line 3—3 Fig. 2.

Like characters of reference denote corresponding parts throughout the figures.

The present invention has to do with the improvement on the process or method of coating and treating materials having an iron base, as disclosed by my Patent No. 1,430,648 dated Oct. 3, 1922; the metal-coated iron or 50 steel article, as disclosed by my Patent No. 1,468,905, and the apparatus for coating and treating metallic materials, as disclosed by my Patent No. 1,580,887 dated April 13, 1926.

My present invention has to do with a vertical hot tube, as distinguished from a horizontally disposed furnace; also the elimination of skimming devices, as well as wipers, with the result that the zinc coating (especially on wire) remains undisturbed while in the 55 molten or semi-molten state, with the result that the thickness of the solid zinc coating, on the finished wire, is very uniform, both diametrically and longitudinally. Furthermore, by submerging the lower end of the so 60 called hot tube in the molten zinc, in the galvanizing pan, ingress of air into the tube, at the surface of the zinc, is prevented. Such an arrangement not only inhibits partially 65 the formation of zinc oxide, on the surface 70 of the zinc coating during heat-treatment, but also inhibits in degree the formation of zinc oxide skimmings on the surface of the molten zinc inside the hot tube, both of which are undesirable.

In the drawings 1 designates a galvanizing pan, of the usual design and structure in which is carried the molten zinc *a* and through which the material to be coated is moved. In the present instance the material 80 illustrated as being coated and subsequently heat-treated is wire *b*, although it is not intended by such disclosure to limit the invention to the coating and heat-treating of wire as the apparatus employed may be made 85 adaptable to the coating and heat-treating of strip and other materials. Primarily, the invention is directed to the zinc coating of materials having an iron or steel base, and the heat-treating of such coated materials.

At a suitable point, over the pan 1, where it is intended to remove the material which has been coated with zinc, there is located or built up or suitably supported a vertical hot tube 2 and said hot tube and its associated elements are supported by a preferably steel structure 3, and such structure preferably comprises the frame of upright beams 4 extending up from the floor or foundation 5 to a point well above the pan 1 and it is into this frame and between these uprights that the pan 1 extends, somewhat in the manner shown in Fig. 1. The uprights are connected at their upper ends by a head frame 6 and the said uprights mediate their upper and lower ends and at a suitable point above the pan 1 are connected by cross-frames 7, in turn jointed by other frame parts 8.

The vertical hot tube 2 is disposed in a vertical position within and in an axial position in relation to the frame composed of the upright beams 4 and the cross-connecting frame parts 7 and 8 with the lower end of the hot tube structure located and supported immediately above the pan 1, see Fig. 2.

The structure constituting the vertical hot tube and the tube proper I prefer to be constituted of and arranged and assembled as follows: A body preferably rectangular in cross-section is enclosed within a metallic casing 9 which comprises side and end walls, a bottom closure and a top closure, see Fig. 2, with the corners, bottom and angular portions suitably braced and reinforced, as at 10, see Figs. 2 and 3. Disposed centrally within the enclosing wall, is the tube 11, which projects through and below the lower wall of the casing and down into the zinc spelter *a* within the pan 1, see Fig. 2 and which also projects through and above the upper wall of said casing, see also Figs. 1 and 2. I prefer, as shown in Fig. 3, that the tube 11 be made of two tubes which shall be oblong or rectangular in cross section and arranged and disposed as shown in Fig. 2 and that each tube shall comprise upper and lower joined sections 12 and 13. The upper sections are preferably of soft steel or like material and the lower sections of suitable heat resisting material. The greater portion of the length of the tubes 11 are disposed within a vertical flue 14, the walls forming which being of a suitable refractory material 15 having lateral flues 16 therethrough at their upper ends which are in communication with other vertically disposed flues 17 disposed between the walls 15 and similar walls 18 of suitable refractory material. The flues 17 at their lower ends communicate with angularly disposed or lateral exhaust flues 19 which open out through the sides of the casing, see Fig. 2. In addition to the refractory walls or linings 15 and 18, which form the flues 14, 16, 17 and 19 and provide insulating members within the casing, there is also provided other linings 20 of

suitable insulating material, as a backing for the sides and ends of the casing and the top thereof. The walls 15 and 18 are separated by the spacers 21 of suitable refractory material. The lower ends of the flues 14 are chambered as at 22 for the introduction of a heating medium which circulates up through the flue 14, across through the flues 16 and down through the flues 17 and out through the exhaust flues 19.

I prefer to heat the hot tube proper by means of a gas flame and to heat-treat the coated material passing through the hot tube by radiation of heat from the tube. Burners 23 project a flame into the chambered end of the flue 14 and said burners are connected, respectively, with piping 24 connected with a suitable source of supply. Any means may be provided to give access to the burners and if the life of the hot tube is too short, by reason of the direct contact of the flame, a baffle of some suitable material may be placed between the tube and burners. The temperature and temperature gradient inside the hot tube would preferably be—800° F. to 1200° F. for the lower hot zone of the hot tube, preferably represented by the tube section 13, and 600° F. to 1000° F. for the upper hot zone, of the hot tube, preferably represented by the tube section 12. These suggested temperatures are not limiting in any sense as they may be varied to meet all conditions of practice. I recommend a predetermined length of hot tube for a given unit, which, however, may be varied in different units and for different materials, as of course will be understood.

In the practical application of the invention, I have elected to show a structure designed for use in connection with the zinc coating of wire and the heat-treating of such material and while any commercial gauge diameter of wire is usable, for rate of travel of the wire through the zinc bath and hot tube, I recommend a range of speed of from thirteen (13) to fifty-two (52) feet per minute. The wires *b* are passed through the molten zinc *a* in the pan 1 and over preferably grooved rollers 25 which are submerged in the molten zinc and carried by a shaft 26 which passes out of opposite walls of the pan 1 and carried or supported by suitable bearings. The wires are guided to and from the rollers 25, by suitable grooved guides 27 and 28 suitably supported submerged in the molten zinc. The wires *b* are guided axially of and through the hot tube in the manner shown in Figs. 2 and 3 and on leaving the hot tube the wires are directed, preferably exposed to the atmosphere to the upper end of the frame structure for the hot tube and over preferably grooved rollers 29, see Fig. 1, carried by a shaft 30 suitably journaled on the head frame 6, and from the rollers 29 the coated and heat-treated wires are di-

rected to the blocks on the take-up frame (not shown) by guiding rollers 31 carried by a preferably downwardly inclined frame 32. The rollers 25 and 29 are preferably so arranged or located with respect to each other 5 that the wire *b* leaving one set and passing through the hot tube to the other set travel vertically, tangent to both sets of rollers and within and parallel with the wall of the hot tube. Furthermore, the disposition of these 10 elements is such that the hot galvanized wire may be carried directly from the molten zinc bath vertically into and through the hot tube or heat-treating chamber without touching the walls thereof (or any other object) 15 until the zinc coating on the wire has been well solidified. It should be apparent, therefore, that by the use of the within described process, made possible by the structure disclosed, that the zinc coated wire does not 20 come into contact with any rigid object either during emergence from the molten zinc (when the surface tension of the molten zinc coating causes it to adhere to the wire as a continuous liquid film of uniform thickness); 25 or while it is passing through the hot tube to effect heat-treatment of the zinc coating; or thereafter until the zinc coating has become completely solidified (after which the 30 wire passes over the upper roller and from thence to the blocks on the take-up frame). Therefore, the zinc coating remains undisturbed while in the molten or semi-molten state, with the result that the thickness of the 35 solid zinc coating on the finished wire is very uniform, both diametrically and longitudinally. Furthermore, due to the fact that there is no zinc removed from the wire by any contact of the coated wire, either during 40 emergence from the bath or after leaving the bath, as for example with drip-bars, skimmers, wipes or the like, it is possible to get the maximum coating of zinc, consistent with the time that the wire is immersed in the 45 zinc bath.

I am familiar with most, if not all, processes and apparatus for zinc coating materials where efforts have been made to obtain uniformity of coatings, including those of my 50 own, to which reference has been made, but in all such processes and apparatus, with which I am familiar such uniformity of coating thickness, both diametrically and longitudinally, has been very difficult to attain; 55 especially where the hot zinc coated wire is pulled over a drip-bar or skimmer as it emerges from the molten zinc bath, and is then carried horizontally through a heat-treater for heat-treatment of the zinc coating.

60 The continuous dragging contact with a drip-bar, skimmer or the like causes a partial wiping of one side of the coated wire, which is only partially alleviated by the effect of surface tension on the semi-molten coating during 65 passage through the heat-treater. The adhesive and bending qualities of the zinc coating after application and heat-treatment as herein pointed out and by the use of the vertical hot tube is directly dependent upon the various factors to which I have heretofore 70 referred.

I have made mention of the submergence of the lower end of the hot tube in the molten zinc which will prevent ingress of air at the surface of the molten zinc, which inhibits 75 partially, if not wholly, the formation of zinc oxide on the surface of the zinc coating during heat-treatment, as well as inhibits in degree the formation of zinc oxide skimmings on the surface of the molten zinc inside the 80 hot tube, both of which are undesirable. In order to reduce the amount of surface oxidation of both the zinc bath and the zinc coating inside the hot tube, a suitable deoxidizer, as for example a thin layer of preferably 85 granular charcoal 33 is used to cover the surface of the molten zinc, in the lower end of the hot tube, see Fig. 2. The deoxidizer or charcoal is applied by dropping it into the hot tube at upper end thereof. This deoxidizer or charcoal layer is not used in any 90 sense as a "wipe", but is used distinctly as a deoxidizer inside the lower end of the hot tube, particularly at the surface of the molten zinc where the coated wire emerges into the 95 hot tube atmosphere.

What I claim is:—

1. The herein described method of zinc coating wire having an iron or steel base and immediately following such coating heat-treating the wire and coating while the coating is in a non-solidified condition, which consists in subjecting the wire to a bath of molten-zinc and removing the coated wire from the bath in a vertical direction and at the same time heat-treating such wire and coating, and in passing the coated wire through a deoxidizer at the point of emergence of the wire from the bath to the zone of heat-treatment, whereby to reduce the 100 amount of surface oxidation of the zinc bath at the surface of the molten zinc where the wire emerges therefrom and also within the heat-treating zone.
2. The herein described method of zinc coating wire having an iron or steel base and immediately following such coating heat-treating the wire and coating while the coating is in a non-solidified condition, which consists in subjecting the wire to a bath of molten-zinc and removing the coated wire from the bath in a vertical direction and at the same time heat-treating such wire and coating, and in passing the coated wire through a thin layer of granular charcoal at the point of emergence of the wire from the bath to the zone of heat-treatment, whereby to reduce the amount of surface oxidation of the zinc bath at the surface of the molten 110 zinc.

105

115

120

125

130

zinc where the wire emerges therefrom and also within the heat-treating zone.

3. In an apparatus of the character described, in combination, a galvanizing pan for use with a bath of molten-zinc, means for diverting material subjected to the bath into a vertical path of travel as such material leaves the bath, a structure supported in a vertical position above the pan at the point where the material emerges from said pan, such structure characterized by having a central vertical heating flue and spaced vertical exhaust flues on opposite sides thereof in communication with said central flue at their upper ends and with exhaust outlets at their lower ends, an imperforate hot tube disposed in vertical position in said central flue through which the coated material is carried and having its lower end projecting through the structure and being submerged in the bath of molten zinc, means to guide the material from the pan and through the tube so as to prevent the material and coating from coming into contact with any object during emergence of the material from the bath and through the tube and until the coating has become substantially solidified, and means for heating the tube through heat inlets at the lower end of said central flue and in turn through radiation of the heat from the tube heat-treating the material and coating as it is carried through the tube.

4. In an apparatus of the character described, in combination, a galvanizing pan for use with a bath of molten-zinc, means for diverting material subjected to the bath into a vertical path of travel as such material leaves the bath, a structure supported in a vertical position above the pan at the point where the material emerges from said pan, such structure characterized by having a central vertical heating flue and spaced vertical exhaust flues on opposite sides thereof in communication with said central flue at their upper ends and with exhaust outlets at their lower ends, an imperforate hot tube disposed in vertical position in said central flue through which the coated material is carried and having its lower end projecting through the structure and being submerged in the bath of molten zinc, means to guide the material from the pan and through the tube so as to prevent the material and coating from coming into contact with any object during emergence of the material from the bath and through the tube and until the coating becomes substantially solidified, means for heating the tube through heat inlets at the lower end of said central flue and in turn through radiation of the heat from the tube heat-treating the material and coating as it is carried through the tube, and a deoxidizing material on the surface of the bath within the tube, where the tube is submerged in the bath, to reduce the amount of surface oxidation of

both the zinc bath and the coating where the coated material emerges into the atmosphere of the tube from such bath.

5. In an apparatus of the character described, in combination, a galvanizing pan for use with a bath of molten-zinc, means for diverting material subjected to the bath into a vertical path of travel as such material leaves the bath, a structure supported in a vertical position above the pan at the point where the material emerges from said pan, such structure characterized by having a central vertical heating flue and spaced vertical exhaust flues on opposite sides thereof in communication with said central flue at their upper ends and with exhaust outlets at their lower ends, an imperforate hot tube disposed in vertical position in said central flue through which the coated material is carried and having its lower end projecting through the structure and being submerged in the bath of molten zinc, said tube consisting of joined aligned vertical sections, certain of which are of heat resisting material and certain others being of the consistency of soft steel, means to guide the material from the pan and through the tube to prevent the material and coating from coming into contact with any object during emergence of the material from the bath and through the tube and until the coating has become substantially solidified, and means for heating the tube through heat inlets at the lower end of said central flue and in turn through radiation of the heat from the tube heat-treating the material and coating as it is carried through the tube.

6. In an apparatus of the character described, in combination, a galvanizing pan for use with a bath of molten-zinc, means for diverting material subjected to the bath into a vertical path of travel as such material leaves the bath, a structure supported in a vertical position above the pan at the point where the material emerges from said pan, such structure characterized by having a central vertical heating flue and spaced vertical exhaust flues on opposite sides thereof in communication with said central flue at their upper ends and with exhaust outlets at their lower ends, an imperforate hot tube disposed in vertical position in said central flue through which the coated material is carried and having its lower end projecting through the structure and being submerged in the bath of molten zinc, said tube consisting of joined aligned vertical sections, certain of which are of heat resisting material and certain others being of the consistency of soft steel, means to guide the material from the pan and through the tube as to prevent the material and coating from coming into contact with any object during emergence of the material from the bath and through the tube and until the coating be-

comes substantially solidified, means for heating the tube through heat inlets at the lower end of said central flue and in turn through radiation of the heat from the tube  
5 heat-treating the material and coating as it is carried through the tube, and a deoxidizing material on the surface of the bath within the tube, where the tube is submerged in the bath, to reduce the amount of surface  
10 oxidation of both the zinc bath and the coating where the coated material emerges into the atmosphere of the tube from such bath.

JOSEPH L. HERMAN.

15

20

25

30

35

40

45

50

55

60

65